

## 1

2,937,993

## HIGH MELTING POINT SYNTHETIC BASE GREASE CONTAINING AN ALKALI METAL SALT OF A DICARBOXYLIC ACID

Warren C. Pattenden, Courtright, Ontario, Lorne W. Sproule, Sarnia, Ontario, and James H. Norton, Corunna, Ontario, Canada, assignors to Esso Research and Engineering Company, a corporation of Delaware

No Drawing. Filed Sept. 23, 1957, Ser. No. 685,395

5 Claims. (Cl. 252—41)

This invention relates to greases and grease thickeners and to methods for their preparation. In particular, it relates to grease compositions comprising a major proportion of a lubricating oil and a thickening amount of a thickener comprising a salt of a dicarboxylic acid and to methods for preparing the grease compositions.

This application is a continuation-in-part of U.S. application Serial No. 605,726, filed August 23, 1956, and now issued as U.S. Patent No. 2,898,296.

Salts of dicarboxylic acids are known to have high melting points but are usually so indispersible in mineral oil that they have found little use in grease manufacture. It has now been discovered that grease thickeners having high dropping points can be prepared by the direct reaction of a metal base with either a dibasic acid ester or with a mixture of an aliphatic dicarboxylic acid and a monohydric aliphatic alcohol. It has also been discovered that excellent grease thickeners can be prepared in a lubricating oil menstruum from a mixture of an aliphatic monocarboxylic acid salt and a metal salt of a dicarboxylic acid, the latter salt being obtained by saponification of the diester of the dicarboxylic acid. The latter thickeners may be prepared by neutralizing a mixture of an aliphatic monocarboxylic acid and a synthetic ester of a dicarboxylic acid with a metal base in either a mineral oil or synthetic oil menstruum. Greases prepared with any of the above grease thickeners are homogeneous in appearance and have exceptionally high dropping points.

The synthetic diesters useful in this invention are those formed by the reaction of an aliphatic dicarboxylic acid and a monohydric aliphatic alcohol. These diesters have the general formula:



wherein R and R<sub>1</sub> are alkyl radicals of either straight-chain or branched-chain aliphatic saturated monohydric alcohols containing about 1 to 22, advantageously 1 to 10 carbon atoms per molecule, and x is a number from 0 to 20, advantageously 4 to 8. The diester molecule will contain a total of about 4 to 64, advantageously 6 to 28 carbon atoms. Also included are diesters prepared from Oxo alcohols, which are an isomeric mixture of highly branched-chain primary alcohols prepared by the "Oxo" process, which is well known in the art.

The aliphatic monocarboxylic acids useful in carrying out the invention are those acids which have about 6 to 30, advantageously 10 to 18 carbon atoms per molecule. These aliphatic monocarboxylic acids may be saturated or unsaturated, straight or branched-chain, and may be hydroxy substituted.

The monohydric aliphatic alcohols used in the mixtures which contain an aliphatic dicarboxylic acid are either

## 2

straight-chained or branched-chained aliphatic saturated monohydric alcohols containing about 1 to 22 and preferably 1 to 10 carbon atoms per molecule.

The aliphatic dicarboxylic acids used in accordance with this invention have the following formula:



wherein x is a number from 0 to 20, advantageously from 4 to 8.

10 Metal bases of any of the metals commonly used in making grease thickeners may be used to neutralize the mixture of an aliphatic monocarboxylic acid and a synthetic ester. Generally used are the alkali metal and alkaline earth metal hydroxides or oxides. These may be used in the form of a hydrate or in water solution.

The metal bases contemplated for use with mixtures not containing an aliphatic monocarboxylic acid are the alkali metal bases lithium hydroxide and sodium hydroxide used in the form of a hydrate or in an aqueous solution. It was found that it was not possible to substitute calcium hydroxide for the alkali metal bases in the process not employing an aliphatic monocarboxylic acid.

The menstruum for preparing the thickeners may be a mineral oil, a synthetic oil, or a synthetic diester oil of the type used to form the thickener. When the menstruum is a synthetic diester oil, only a portion of the synthetic diester is converted into the thickener, depending upon the amount of metal base which is used. After the grease thickener is formed by the reaction with a metal base, additional mineral oil, or additional synthetic ester oil, or even additional amounts of any of the other known synthetic oils may be added to form the final grease composition.

30 The grease cooking temperature is generally determined by the boiling point of the alcohol which is added to the mixture or formed by the saponification of the diester, depending on which variation of the process is used. The presence of too much alcohol in the final grease reduces the yield and dropping point appreciably. It is therefore desirable to cook the grease sufficiently to remove the alcohol which is added or which is formed during the process. Generally used are temperatures of about 300 to 500° F., preferably 300 to 400° F. Lower temperatures can be used if the alcohol is removed under reduced pressure. The mixture is then heated for a period of time sufficient to complete the neutralization of the acids, form the thickener, and to evaporate the alcohol. This period of time will generally be about 5 to 120 minutes, usually 10 to 30 minutes.

45 Additional lubricating oil and additives may be added to form the final grease product. The grease may then be homogenized through a Manton-Gaulin homogenizer or a similar type of homogenizer, and packaged.

55 The grease compositions of the invention consist of a major proportion, 60 to 95 wt. percent, preferably 75 to 93 wt. percent, of a lubricating oil and a thickening amount, about 5 to 40 wt. percent, preferably 7 to 25 wt. percent of the grease thickener. The grease thickener containing an aliphatic monocarboxylic acid comprises about 20 to 80 wt. percent, preferably 30 to 70 wt. percent of the aliphatic monocarboxylic acid salt and about 80 to 20 wt. percent, preferably 70 to 30 wt. percent of the dicarboxylic acid salt.

60 65 The invention will be better understood by the following illustrations which include the preferred embodiments of the invention.

The following Examples I through VIII and Tables I and II are illustrative of grease compositions prepared by the direct reaction of a metal alkali with a dibasic acid ester or with a mixture of an aliphatic dicarboxylic acid and a monohydric aliphatic alcohol without the presence of an aliphatic monocarboxylic acid soap. Examples X through XVI and Table III are illustrative of grease compositions containing a mixture of an aliphatic monocarboxylic acid soap and a metal salt of a dicarboxylic acid.

### EXAMPLE I

A grease was prepared by mixing 15 grams of di-(2-ethyl hexanol) sebacate with 81.7 grams of a silicone lubricating oil having a viscosity at 100° F. of 475 cst. and a V.T.C. of 0.83. 3.3 grams of LiOH.H<sub>2</sub>O were added and the mixture was then heated to a temperature of about 400° F. and maintained at this temperature for about 15 minutes. The 2-ethyl hexanol which formed during the reaction was driven off almost as rapidly as it formed. The grease was then cooled and inspected.

### EXAMPLES II TO IV

Additional greases were prepared in the manner described in Example I using the ingredients as noted in Table I. The composition of the greases of Examples I through IV and their characteristics are likewise shown in Table I.

Table I

| Example Number.....                         | I    | II   | III  | IV    |
|---------------------------------------------|------|------|------|-------|
| Composition in grams:                       |      |      |      |       |
| Di-2-ethyl hexyl sebacate.....              | 15.0 |      |      | 30.0  |
| Diethyl sebacate.....                       |      | 33   | 33   |       |
| LiOH.H <sub>2</sub> O.....                  | 3.3  | 10   |      | 6.6   |
| NaOH.....                                   |      |      | 10   |       |
| Dow Corning Fluid 710 <sup>1</sup> .....    | 81.7 | 57   | 57   |       |
| Mineral Oil <sup>2</sup> .....              |      |      |      | 64.0  |
| Inspections:                                |      |      |      |       |
| ASTM micropenetration, mm./10 at 77° F..... | 80   | 74   | 48   | 400+  |
| Dropping Point, ° F.....                    | 500+ | 580+ | 580+ | ----- |

<sup>1</sup> Dow Corning Fluid 710 is a silicone fluid having a viscosity at 100° F. of 475 cst. and a V.T.C. of 0.83.

<sup>2</sup> A solvent treated and dewaxed Canadian distillate having a viscosity at 100° F. of 550 S.U.S., and a V.I. of 90.

The following greases are examples of the process using an aliphatic dicarboxylic acid and a monohydric aliphatic alcohol as starting materials in place of the above diesters. These greases can be prepared by slowly adding an aqueous solution of the alkali to the acid and alcohol dissolved in lubricating oil or the dicarboxylic acid can be dissolved and/or dispersed in a suitable volatile solvent such as 2-ethyl hexanol or water, and this solution then added to an aqueous alkali, alcohol, lubricating oil mixture.

### EXAMPLE V

A grease was prepared by mixing 20 grams of adipic acid and 36 grams of 2-ethyl hexanol with 100 grams of a silicone lubricating oil having a viscosity at 100° F. of 100 cst. and a V.T.C. of 0.78. 11 grams of LiOH.H<sub>2</sub>O dissolved in water were added and the mixture was then heated to a temperature of about 400° F. and maintained at this temperature for about 15 minutes in order to complete the reaction and drive off the water and alcohol. The grease was then cooled and inspected.

### EXAMPLES VI TO VIII

Additional greases were prepared in the manner described in Example V using the ingredients as noted in the following Table II. The compositions of the greases of Examples V through VIII and their characteristics are shown in the following table.

### Table II

| Example Number.....                      | V     | VI    | VII   | VIII  |
|------------------------------------------|-------|-------|-------|-------|
| Composition in grams:                    |       |       |       |       |
| Adipic acid.....                         | 20.0  |       | 20.0  | 30.0  |
| Sebacic acid.....                        |       | 26.0  | 26.0  | 50.0  |
| 2-ethylhexanol.....                      | 36.0  |       | 36.0  |       |
| LiOH.H <sub>2</sub> O.....               | 11.0  | 8.0   | 12.0  | 12.0  |
| Dow Corning Fluid 550 <sup>1</sup> ..... | 100.0 | 100.0 | 100.0 |       |
| Mineral Oil <sup>2</sup> .....           |       |       |       | 100.0 |
| Inspections:                             |       |       |       |       |
| ASTM micropenetration mm./10.....        | 311   | 165   | 204   | 115   |
| ASTM dropping point.....                 | 500+  | 500+  | 500+  | 500+  |

<sup>1</sup> Dow Corning Fluid 550 is methyl phenyl polysiloxane fluid having a flash point of 575° F. and a viscosity of 100 cst. at 100° F.

<sup>2</sup> A mineral oil having a viscosity of 300 S.S.U. at 100° F. and a V.I. of 70.

In order to show that the salt of a dibasic acid and the soap of an aliphatic carboxylic acid does not form the same type of thickener as the saponified mixture of an aliphatic carboxylic acid and diester or alcohol-dicarboxylic acid mixtures, the following experiment was made.

### EXAMPLE IX

A grease was prepared by heating 10 wt. percent stearic acid, 4.8 wt. percent sebacic acid, 3.6 wt. percent LiOH.H<sub>2</sub>O (sufficient LiOH.H<sub>2</sub>O to neutralize both acids) and mineral oil, to 300° F. This grease had a dropping point of 360° F. and contained most, if not all, of the lithium sebacate as coarse visible particles. Attempts to disperse or redisperse the salt of the dicarboxylic acid, once it had separated into the grainy state, have been unsuccessful, even when the grease was heated to 500° F. Since the dropping point of lithium stearate grease is about 370° F., it is apparent that little or no lithium sebacate has been codispersed with the soap.

### EXAMPLE X

A grease of the invention was prepared by mixing 10 grams of stearic acid and 10 grams of di-2-ethyl hexyl sebacate (equivalent to 4.8 grams of sebacic acid) with 80 grams of a mineral lubricating oil having a viscosity at 100° F. of 300 S.U.S. and V.I. of 70. 3.6 grams of LiOH.H<sub>2</sub>O were added and the mixture was then heated to a temperature of about 400° F., and maintained at this temperature for about 15 minutes. The 2-ethylhexanol which formed during the reaction was driven off almost as rapidly as it formed. The grease was then cooled and inspected.

### EXAMPLES XI TO XV

Additional greases of the invention were prepared in the manner described in Example X using the ingredients as noted in Table III. The compositions of the greases of Examples X through XV, and their characteristics, are also shown in Table III.

### EXAMPLE XVI

A grease of the invention was prepared by mixing 13.7 parts by weight of stearic acid and 19.4 parts of diethyl adipate (equivalent to 14.0 parts of adipic acid) with 58.2 parts of Diol 50 at a temperature of 200° F. in a Manton-Gaulin homogenizer. The mixture was circulated through the homogenizer and a water slurry containing 8.7 parts of calcium hydroxide was added. The resultant mixture was then circulated for 6 hours at temperature of 200° F. and a pressure of 2,000 lbs. Thereafter, the grease was removed and transferred to a grease kettle where it was dehydrated at a temperature of 400° F. The grease was then cooled and inspected.

Table III

| Example Number                                         | IX   | X    | XI   | XII  | XIII | XIV  | XV   | XVI  |
|--------------------------------------------------------|------|------|------|------|------|------|------|------|
| Composition in grams:                                  |      |      |      |      |      |      |      |      |
| Stearic Acid                                           | 10.0 | 10.0 | 10.0 | 10.0 | 10.0 | 10.0 | 10.0 | 13.7 |
| Sebacic Acid                                           | 4.8  |      |      |      |      |      |      |      |
| Di-2-ethyl hexyl sebacate                              |      | 10.0 | 10.0 |      |      | 10.0 | 10.0 |      |
| Di-2-ethyl hexyl adipate                               |      |      |      | 10.0 | 10.0 |      |      |      |
| Diethyl adipate                                        |      |      |      |      |      |      |      | 19.4 |
| LiOH, H <sub>2</sub> O                                 | 3.6  | 3.6  |      | 3.9  | 4.0  | 4.0  | 4.0  |      |
| NaOH                                                   |      |      | 3.8  |      |      |      |      |      |
| Ca(OH) <sub>2</sub>                                    |      |      |      |      |      |      |      | 8.7  |
| Mineral Oil (Viscosity at 100° F.<br>300 SUS; V.I. 70) | 80.0 | 80.0 | 51.0 | 80.0 | 20.0 | 80.0 |      |      |
| Ucon LB-1800X <sup>1</sup>                             |      |      |      |      | 60.0 |      |      |      |
| Di-2-ethyl hexyl adipate (as oil)                      |      |      |      |      |      |      |      |      |
| Dow Corning Silicone Fluid 500 <sup>2</sup>            |      |      |      |      |      | 76.0 |      |      |
| Diol 50                                                |      |      |      |      |      |      | 58.2 |      |
| Inspections:                                           |      |      |      |      |      |      |      |      |
| ASTM penetration, 77° F.                               | 320  | 250  | 220  | 270  |      |      |      |      |
| ASTM wkd. penetration, 77° F.                          | 350  | 265  | 265  | 310  | 340  | 300  | 250  | 273  |
| ASTM Dropping Point, ° F.                              | 360  | 500  | 500+ | 485  | 479  | 600+ | 540+ | 450+ |
| Appearance                                             | (3)  | (4)  | (4)  | (4)  | (4)  | (4)  | (4)  | (4)  |

<sup>1</sup> Ucon LB-1800X is a water-insoluble polyalkylene glycol type of lubricating fluid which is predominantly polypropylene glycol, and has a viscosity at 100° F. of 1800 SUS.

<sup>2</sup> Dow Corning Silicone Fluid 550 is a phenyl methyl polysiloxane having a flash point of

575° F. and a viscosity at 25° C. of about 100 to 150 centistokes.

<sup>3</sup> Many Undispersed Particles

<sup>4</sup> Homogeneous.

As seen from Table III, the greases of the invention (X through XVI) had very high dropping points of from above 450° F. to above 540° F. and formed homogeneous products. However, the grease formed by the neutralization of the stearic acid and sebacic acid (IX) had a dropping point of only 360° F. and contained many undispersed particles.

Various other additives may be added to the grease composition of the invention, such as oxidation inhibitors, dyes, metal deactivators, corrosion inhibitors, deodorants, and so forth, as understood by those skilled in the art.

What is claimed is:

1. A process for preparing a lubricating grease composition comprising a major proportion of a lubricating oil and about 5 to 40 wt. percent of an alkali metal salt of a dicarboxylic acid which comprises heating a mixture of an alkali metal base, lubricating oil, an aliphatic dicarboxylic acid containing from 2 to 22 carbon atoms per molecule and a monohydric aliphatic alcohol having from 1 to 22 carbon atoms per molecule, said heating taking place at a temperature in the range of 300° to 500° F. for a time sufficiently to form said metal salt and to evaporate said alcohol.

2. A process according to claim 1 wherein said lubricating grease composition comprises about 60 to 95 wt. percent of said lubricating oil and about 40 to 5 wt. percent of said thickener.

25 3. A process for preparing a lubricating grease composition having 60 to 95 wt. percent of a lubricating oil and 40 to 5 wt. percent of an alkali metal salt of a dicarboxylic acid which comprises heating to a temperature in the range of 300° to 500° F. for a time in the range 30 of 5 to 125 minutes, a mixture of (1) an alkali metal base, (2) a lubricating oil, and (3) a mixture of a C<sub>2</sub> to C<sub>22</sub> aliphatic dicarboxylic acid and a C<sub>1</sub> to C<sub>22</sub> mono-hydric aliphatic alcohol, said heating being sufficient to form said metal salt and to remove substantially all of 35 said alcohol.

4. A process according to claim 3 wherein said alkali metal base is used in an aqueous solution.

5. A process according to claim 3 wherein said metal base is taken from the group consisting of lithium hydroxide and sodium hydroxide.

#### References Cited in the file of this patent

#### UNITED STATES PATENTS

|           |                   |               |
|-----------|-------------------|---------------|
| 2,363,514 | Farrington et al. | Nov. 28, 1944 |
| 2,528,373 | Knowles et al.    | Oct. 31, 1950 |
| 2,583,607 | Sirianni et al.   | Jan. 29, 1952 |
| 2,699,428 | Lux et al.        | Jan. 11, 1955 |
| 2,710,838 | Morway et al.     | June 14, 1955 |
| 2,801,220 | Smith             | July 30, 1957 |